

Sept. 18, 1934.

R. KAUFHOLD

1,974,334

PROCESS OF COLORING SILVER IMAGES

Filed Sept. 26, 1932

Fig. 1.



Fig. 2.



Fig. 3.



INVENTOR.  
R. Kaufhold  
BY: Marks & Clark  
ATTORNEYS.

## UNITED STATES PATENT OFFICE

1,974,334

## PROCESS OF COLORING SILVER IMAGES

Robert Kaufhold, Feldkirch, Austria, assignor to  
the firm Koh-I-Noor-Bleistiftfabrik L. & C.  
Hardtmuth, Ceske Budejovice, Czechoslovakia

Application September 26, 1932, Serial No. 634,981  
In Germany August 30, 1929

4 Claims. (Cl. 95—5)

The present invention relates to a process of coloring silver images and particularly to a process of coloring photographic positives and negatives.

Hitherto silver images were colored with transparent colors or covering dyes. When these known coloring processes are used it is, however, not possible to reproduce the light and dark shades correctly, since the grey silver particles will shine through the layer of colors, whereby images 5 pure tones are produced. Moreover, when working after these known methods, it would be necessary, in order to obtain satisfactory results, to color the areas of different light values individually and with utmost care. This coloring 10 method is, however, hardly practicable and usually, therefore, for instance the leaves of clumps of trees or bushes are simply painted green without regard to the fact, that each single leaf comprises a plurality of color shades. Therefore, 15 even carefully painted photographic prints will never be a really artistic reproduction of nature. 20

The object of the present invention is to provide a simple and practical process for producing colored pictures from photographic prints which 25 will give better results than the processes hitherto known.

According to the present invention, in carrying out a process of the kind referred to above, the coloring is performed by applying pigments to a photographic negative or positive, coating the pigments with a layer of colored or uncolored colloid and bleaching and washing the picture. Through this treatment the surplus of pigments and of gelatine is removed. Thereupon the white 30 silver image is fixed out and the picture is washed. The product obtained is a pure colored picture. 35

When a photographic positive is to be colored the process may be carried out in the following manner:

The print is painted roughly with powdered pigments, pencil colors or other pigment solutions in which no colloid is present. Pigment solutions are not so-called genuine color solutions, as for instance, anilin color substances diluted in water, but insoluble color substances finely divided in benzine, turpentine oil, etc., which volatilize after application, leaving the dry powder color behind. Hereby no regard is taken to light and dark tones or shades. Groups of houses are, for instance, simply colored brown or yellow, woods and meadows green and the sky blue. The painted print is coated with a layer of colloid, preferably of colored or uncolored gelatine. If the print is colored only with light pigments, it is 40 coated with a dark colored gelatine solution. If, 45

however, besides light colors also black pigments or dark colors are applied to the darker areas of the picture, the print is covered with an uncolored gelatine solution. The print may now be dried, but it is also possible to continue the treatment 80 with prints in damp state. The print is thereupon bleached. Suitable bleaching agents are, for instance, the solutions used by the preparation of bromoil- and ozobromium prints. Solutions of this kind will penetrate all layers and convert the 85 blackened silver of the original image into white silver. Simultaneously the ozobromium content of the bleaching agents will cause a hardening of the pigment layers superimposed on the silver image in accordance with the image proper. The 70 product is thereupon washed with tepid water. During the washing procedure such colored layers as still remain soft will be separated from the picture. The picture is now treated with a soft brush and simultaneously the picture may be re-touched, if desired. Finally the product is fixed 75 and washed in the usual way.

Instead of painting the picture with pencils or solutions of pulverulent pigments the dyeing 80 may be performed by means of colored or tinged, regular or irregular crystals or circles, pencils or carbons, bronze colors, short colored silk threads and the like.

The essential feature of the present process 85 consists in the fact that the original image (the finished silver image) is at first colored with powdered or pencil colors as a single or multi-colored picture, upon which the colloid, for instance, gelatine and preferably a dark colored gelatine, is poured or spread.

The process is shown diagrammatically in the accompanying drawing in which Figure 1 indicates the silver image before bleaching; Fig. 2 after bleaching and Fig. 3 the completely fixed image. 90

The following takes place: In the process of pouring or spreading, see Fig. 1, the dark liquid layer of gelatine moistens the dry powdered color lying underneath down to the bottom. Therefore, by the penetration of the gelatine into the 100 dry red or other powdered color, a red glue layer and above it a dark glue layer lies on the silver image.

In addition to this is a special characteristic of the process: The red layer of the powdered 105 color forms, as it were, a screen for the dark layer of gelatine lying above it. It absorbs the liquid gelatine, but not the gross coloring particles contained therein. Therefore, the tone of the red glue layer remains pure. 110

But it is not always necessary to use a dark colored glue layer although in most cases such a dark colored glue layer is applied. For certain purposes, another tone may be employed and 5 even a completely plain or colorless layer of glue.

Contrary to other processes in which the initial silver image is brought into contact with the already colored layers of colloid, the present process is carried out in a separate manner i. e., at 10 first the pigment is applied and then the layer of glue, whereupon both layers are united.

This is the essential feature of the process. It is presumed that the further treatment is already known.

15 Thereupon follows the bleaching and tanning of the silver image and therewith the tanning of the colored layers of gelatine lying above it and the removal of the untanned parts in a bath of warm water. There remains then a colored 20 image of gelatine as shown in Figure 2. The delicate graduations are reproduced by light colors, as in the example by red, the middle densities by red and a small amount of black, and the 25 shadings by a higher amount of black but in which the red ground shines through.

In this way it is possible to produce a multi-colored image i. e., an image in which the colors appear as in nature. When, for instance in a 30 landscape, the sky is to be reproduced in a blue color, the woods and meadows in a green color etc., water colors are not suitable for this purpose. It is true, they already contain the necessary 35 colloid, glue or albumin, but it is not possible to apply the colors in a completely equal manner one with the other. This is only possible when carried out as in the present process i. e., when 40 at first, the coloring is effected by means of pastel colors or with the pastel crayon and only when the colloid is added, as above described, by pouring or spreading it on the layer of colors.

Lazur-colors are transparent colors.

In Fig. 3 the completely fixed image is shown.

When coloring by means of fatty pigments the process may be performed in a manner now to be described, whereby an engraving-like effect is obtained: The fatty pigments are applied to the picture in the form of dashes or dots, whereupon the silver layer between the dashes or dots is bleached and the layer of fatty matter is removed by means of benzene. The picture is thereupon treated in the manner described above.

I claim:—

1. A process of coloring silver images comprising the steps of painting the image with suitable pigments, coating it with a layer of colloid, then bleaching it so that the colloid layers on the image become hardened in accordance with the original image, washing away the soluble colloid and fixing out the bleached silver.

2. A process of coloring silver images comprising the steps of painting the image with suitable pigments, coating it with a layer of colored colloid, then bleaching it so that the colloid layers on the image become hardened in accordance with the original image, washing away the soluble colloid and fixing out the bleached silver.

3. A process of coloring silver images comprising the steps of painting the image with suitable pigments, coating it with a layer of an uncolored colloid, then bleaching it so that the colloid layers on the image become hardened in accordance with the original image, washing away the soluble colloid and fixing out the bleached silver.

4. A process of coloring silver images comprising the steps of painting the image with a plurality of layers of suitable pigments, coating it with a layer of colloid, then bleaching it so that the colloid layers on the image become hardened in accordance with the original image, washing away the soluble colloid and fixing out the bleached silver.

ROBERT KAUFHOLD.

45

120

50

125

55

130

60

135

65

140

70

145

150

80

85

90

95

100

105

110

115

120

125

130

135

140